

S. P. M. TASKER.

METHOD OF MANUFACTURING WELDED WROUGHT METAL TUBING.

No. 91,791.

Patented June 22, 1869.



Witnesses:  
James Nicholson  
Robt. Briggs

Inventor:  
Stephen P. M. Tasker

# United States Patent Office.

STEPHEN P. M. TASKER, OF PHILADELPHIA, PENNSYLVANIA.

Letters Patent No. 91,791, dated June 22, 1869

## IMPROVED METHOD OF MANUFACTURING WELDED WROUGHT-METAL TUBING.

The Schedule referred to in these Letters Patent and making part of the same.

Be it known that I, STEPHEN P. M. TASKER, of Philadelphia, in the county of Philadelphia, and State of Pennsylvania, have invented a new and improved Method of Manufacturing Wrought-Metal Tubing; and I do hereby declare the following is a full and exact description thereof, reference being had to the accompanying drawings, making part of this specification, in which—

Figure 1 is a front elevation,

Figure 2 is a side elevation, and

Figure 3, a top view of one form of machine adapted to my method of making tubes.

The letters of reference upon all the drawings relate to corresponding parts.

To enable others skilled in the art to have a full comprehension of my invention, I will proceed to describe the construction and operation of the particular form of machine shown in the drawings, where—

A A is a frame, or stand;

B B are pedestals, or bearings;

C C are spur-gear wheels;

D D are mitre-gear wheels;

E E or F F are, either one or the other of them, as most convenient for the application of power, main driving or transmitting-shafts;

G G are roll-shafts;

H H are rolls; and

I I is the mandrel, which mandrel is supported, at one end, by a stand, not shown on the drawings.

The pedestals, or bearings of the several shafts are provided with adjustments, not shown on the drawings, by means of screws, wedges, or other devices well known to mechanics; and the shafts have collars, or steps, whereby the rolls can be set, in the performance of the work. As these means of adjustment present nothing of novelty, and are readily understood, no further description of them is deemed essential at this place.

The outer end of the mandrel I I, which is carried by the stand, (not shown on drawings,) is so far distant from the rolls H H as to allow the finished tube to pass over the mandrel, while the inner end of the mandrel, which shapes, or forms the inside of the tube, is placed in the openings made by the grooves of the rolls. Where the mandrel lays in the grooves, there is a slight enlargement of the body, at K K, so that, in the process of making, the tube fits loosely on the rest of the mandrel after the grooves are passed.

The end of the mandrel is also separate from the stem, at L L, so that it can be drawn from the tube after its completion, by the removal of the end K K. This construction of mandrel is the one usually adopted in rolling tubes with a mandrel, as applied to tubes made with a lap-weld.

In making tubes with a but-weld, except where it is desirable to thin the metal of the tube, no mandrel whatever is required or used.

The mode of operation of the machinery shown on

the drawings, consists merely in giving a rotary motion, in one or the other direction, to the driving-shaft E or F. It will be noticed that this arrangement places two pairs of rolls, one pair in advance of the other, with their axes in planes, at right angles, so that the bite upon the metal between the first pair of rolls and the mandrel, or the compression of the tube, if no mandrel is used, is quartering with the bite, or compression which the second pair of rolls will produce.

To give a full understanding of the nature of my invention, I will state, as briefly as possible, the action of rolls upon the tube, or skelp which forms the tube, where two or more rolls which converge about the tube, having their axes in the same plane, are used, with or without a mandrel in the combination, being the commonly-practised method of manufacturing tubes, both in this country and in England. In this explanation I will again refer to the drawings, in which—

Figure 4 shows a section of the unbent sheet of metal, technically known as a skelp, from which a tube is made;

Figure 5 shows a section of the bent skelp, as prepared for welding in the rolls; and

Figure 6 shows a section of the unfinished tube, when rolled by two rolls.

The skelp has parallel edges, which have been scarfed, or bevelled away the entire length, when lap-welded tubes are to be made, but has square, sound edges when but-welded tubes are to be made. It is bent up, from the form shown in fig. 4, into that shown by fig. 5, as a preliminary operation to the welding in the rolls, at a heat much below a welding-heat. It is then permitted to cool and cast off the scale, or film of oxide which has been formed by exposure of the metal, at the bending-heat, to the air.

To weld on the bending-heat, or bend on the welding-heat, has been found impracticable, although such schemes have been proposed and patented. The surfaces to be welded must be brought in contiguity free from scale.

Contact with the air, or with cold iron, will reduce the temperature of the metal below that at which the scale will fuse away, and the weld be unsound, if not entirely defective. It is even impossible to save the heat of bending by replacing the skelp when bent in the welding-furnace, as the scale formed by exposure to the air then melts off, and, forming a flux for the bottom of the furnace, not only destroys the furnace, but gathers as a glass on the sides of the skelp, forming lumps, which make indentations on the tube when passing the rolls.

The form shown in fig. 5 is that of a loose scroll, with the edges overlapping each other a little more than the width of the beveling, or, generally, about three times the thickness of the metal, so that there is a double thickness of metal at the unwelded joint, (with thinned edges,) to be compressed, when at a weld.

ing-heat, to the same thickness as the rest of the skelp, or tube, when finished.

The enlargement K of the cylindrical mandrel, where the rolls act on the tube, exactly fills the skelp.

The grooves in the rolls, for about one hundred and twenty degrees or to one hundred and fifty degrees, at the bottom, are concentric with the mandrel, and allow the same space for the metal that the tube demands for its thickness all around when finished; the remainder of the grooves—the sides, so to speak—is opened out, to allow the iron to spread, while the corners of the grooves are rounded, so that they shall not mark or cut the tube while it passes through the rolls and over the mandrel.

The entire space between the rolls and the mandrel is just as much less than a section of the skelp, when bent, as it is found practicably possible for the draught of the rolls to pull the skelp over the mandrel without sticking. It follows that a section of a tube, after its first or welding-heat, is that shown on fig. 6, and can be compared to that of a Roman capital letter O, (supposing the hole to be circular,) with two ribs, or fins, formed partly by the corners of the grooves in the rolls, and partly by a thin sheet squeezing out on the faces of the rolls.

Great care is needed to enter the lap of the skelp into the rolls so that the bite shall come upon it, and it is very desirable that the skelp should not twist, as in this case a portion of the lap will come in the parting of the rolls, when a sound weld is by no means so well insured.

This imperfect tube is then permitted to cool, and cast off its scale, for the same reason that the bent skelp is cooled; and is then reheated, and again passed through the rolls, taking care to enter the thick sides, so that the work will now come on them. The fins are either burned or fused away in the furnace, or are so softened as to roll down and weld to the body of the tube, and the tube will be of uniform thickness. In this second rolling, not so much work is put upon the iron between the mandrel and the rolls, consequently little or no fin is formed. The same difficulty of turning down is here encountered, and frequently a third or fourth rolling is needed to get a sound or a uniformly-thick tube. It is possible to make and finish tubes at one rolling, if the inequality of thickness referred to is not regarded, and if the fins be chipped, milled, or pared away.

With inferior iron, (the lower grades of iron being softer when hot,) the grooves in the rolls can be made more nearly concentric than I have described, and the fin only is very objectionable.

With three or four rolls converging together, having their axes in the same planes, the forms of the grooves

can be made altogether concentric to the mandrel, but the fins produced by the partings are not only more in number, but they are more objectionable in size than with two rolls. With this arrangement of three or four rolls, it is nearly impossible to obliterate the fins by re-rolling.

In rolling but-welded tubes without a mandrel, the action of the rolls upon the tube is very nearly as with a mandrel, except that some portion of the effect is expended in making the hole or bore of the tube slightly oval. In but-weld tubes the thickness of metal relative to the diameter is necessarily so great that it acts as a mandrel to a considerable extent.

The improved method of welding, sizing, and smoothing wrought-metal tubes, which I have invented, offers the means whereby, if any fin or inequality of thickness has been formed in the first pair of rolls, it is rolled down and obliterated by the second pair; or if the skelp has twisted, so that the lap has not been brought under the bite of the first pair of rolls, such portion is immediately acted upon by the second pair of rolls, and the weld, the thickness, and the uniformity of the tube is thus insured.

I am aware that four converging rolls, or more than two rolls, with their axes in the same plane, have been proposed and used in welding and sizing tubes. I am aware that two pairs, or a series of pairs of rolls, in advance of each other, with the axes of each pair in planes at right angles, have been proposed for bending up metal forms, and in one or more instances the combination of bending with welding-tubes, by similar series of rolls, has been proposed. I am aware that a pair of rolls, combined with a pair of milling cutters, rotating at right angles to the rolls, to remove the fin, has been proposed. I am aware that two pairs of rolls, with the axes of each pair in planes at right angles, one pair in advance of the other, have been proposed and used, under the name of universal mills for rolling sheet, band, or girder-iron. I am aware that series of pairs of rolls, in advance of each other, with axes of the following pairs at right angles, have been proposed and used in rolling rods and bars. I do not claim any of these machines, nor the application of them to the various processes mentioned; but

What I claim as my invention, and desire to secure by Letters Patent, is—

The method of manufacturing wrought-metal welded tubing from skelps previously prepared by bending, as hereinbefore described.

STEPHEN P. M. TASKER.

Witnesses:

JAMES NICHOLSON,  
ROBT. BRIGGS.